

F. C. GRIMES.

PROCESS FOR RECOVERING POTASSIUM SALTS FROM ORGANIC CARBONACEOUS MATERIALS.

APPLICATION FILED AUG. 19, 1916.

1,227,781.

Patented May 29, 1917.

2 SHEETS—SHEET 1.

Trig. I



### Inventor

F.C. GRIMES

334 Watson E. Coleman

Attorney

F. C. GRIMES.

PROCESS FOR RECOVERING POTASSIUM SALTS FROM ORGANIC CARBONACEOUS MATERIALS.

APPLICATION FILED AUG. 19, 1916.

1,227,781.

Patented May 29, 1917.

2 SHEETS—SHEET 2.



Trig. 2

Inventor

E. C. GRIMES

By Watson E. Coleman

Attorney

# UNITED STATES PATENT OFFICE.

FRANKLIN C. GRIMES, OF IDAHO FALLS, IDAHO.

## PROCESS FOR RECOVERING POTASSIUM SALTS FROM ORGANIC CARBONACEOUS MATERIALS.

1,227,781.

Specification of Letters Patent. Patented May 29, 1917.

Application filed August 19, 1916. Serial No. 115,864.

To all whom it may concern:

Be it known that I, FRANKLIN C. GRIMES, a citizen of the United States, residing at Idaho Falls, in the county of Bonneville 5 and State of Idaho, have invented certain new and useful Improvements in Processes for Recovering Potassium Salts from Organic Carbonaceous Materials, of which the following is a specification, reference being 10 had to the accompanying drawings.

This invention relates to an improved process for recovering potassium compounds from sage brush, seaweed, straw, or other organic carbonaceous materials.

15 It is the primary purpose of the present invention to provide an improved process or method of burning sage brush and similar organic vegetable material wherein an ample supply of oxygen is permitted for facilitating combustion, and the volatilization of the potassium compounds is prevented and the same is retained in the residue or ash instead of being carried off with the products of combustion and dissipated.

25 In the operation of the processes now known in the art for recovering mineral salts and more particularly potassium salts from kelp or seaweed, the total net percentage of the potassium salts remaining 30 in the residue after combustion never exceeds 8%. By means of my improved process which I shall presently describe in detail, the available potassium salts remaining in the residuary ash obtained from sage brush, will vary from 20 to 35%, and for 35 other organic materials in percentages correspondingly greater than is possible under the old processes.

The essential feature of the present invention, whereby this greatly increased percentage of potassium salts is obtained, resides in the addition of sulfur or sulfuric acid to the material either before or during the burning thereof. I have found that the 40 sulfur acts to preserve and retain the potassium salts in the residuary ash so that substantially all of the potassium salts contained in the material is recovered, this being particularly true when the burner is operated under a restricted or repressed draft.

In the accompanying drawing, wherein I have, for the purposes of this explanation, illustrated a type of light, portable burner which I have found admirably adapted for 50 use in the practice of my improved process,

Figure 1 is a longitudinal sectional view through the burner; and

Fig. 2 is a transverse section thereof.

The burner preferably consists of a body having opposed, upwardly diverging, corrugated side walls 5 of cast iron or other suitable heat-resisting materials. To the lower edge of each of these walls, the parallel, longitudinally extending angle bars 6 are securely riveted or bolted. The upper edges 65 of a transversely curved bottom wall 7 are secured between the downwardly projecting, parallel flanges of the respective pairs of angle bars. 8 designates the supports for the burner body which are arranged upon 70 each side thereof, said supports preferably consisting of metal piping. The central portion of each of the pipes extends in parallel relation to the burner body and in a plane below the lowest point of the bottom wall 7. 75 The opposite end portions of the pipes 8 are upwardly inclined and then longitudinally extended, as at 9, beneath the laterally projecting flanges of the outer angle bars 6 to which the pipe ends are bolted or riveted. 80 Superposed, transverse bars 10 extend beneath the bottom wall 7 and in contact therewith and have their end portions obliquely inclined outwardly in diverging relation, as at 11, and the lower ends disposed upon opposite sides of the respective pipes 8 at the ends of the horizontal portions of said pipes. The supporting legs or standards are securely fixed to the pipes by means of the 85 bolts indicated at 12.

A suitable grate 13 is secured to or supported upon the laterally projecting flanges of the inner angle bars 6, and beneath this grate, in spaced relation thereto, a wire screen 14 of not greater than twenty gage, is 90 disposed, the opposite edge portions of the screen being extended upwardly and fixed to the angle bars 6.

The draft may be supplied to the bed of material on the grate through the medium 100 of a plurality of perforated pipes 15 which extend longitudinally between the grate and the screen 14, any suitable means being employed for controlling and regulating the air draft. It is to be particularly observed that 105 the top of the burner body is entirely open so that oxygen may freely enter to the interior of the burner; whereby the combustion of the material will be facilitated.

In carrying out my improved process, the 110

carbonaceous vegetable material, such as sage brush, wood, straw, or seaweed, is fed into the open top of the burner upon the grate 13. The draft supplied through the pipes 15 may be entirely cut off or reduced, as desired. The material, before it is ignited, is treated by sprinkling the same with a solution of sulfuric acid, or particles of sulfur in dry form may be added to the material while burning. The action of the heat upon the sulfur or sulfuric acid liberates sulfur oxid gases which penetrate through the material being burned and convert the potassium salts present in the material as chlorids into sulfates. The latter not being of a volatile character are more readily recovered or saved. Without eliminating or restricting the forced draft beneath the grate and using the sulfur or sulfuric acid as above explained, the mineral salts and especially potassium existing in the carbonaceous material as chlorids, escapes at the temperature necessary for burning the material. As the material burns, the heat tends to drive off the sulfur oxid gases which, if excessive, is abated or reduced by adding a small quantity of common salt to the burning material. When the burning of the material is completed, the potassium salts remaining in the residuary ash consists of potassium carbonate and potassium sulfate. After the material has been completely burned or incinerated, the ash falls through the grate upon the wire screen 14, through which it sifts into the ash pit. All unburned foreign matter is retained upon the screen 14. The ash is then removed from the pit and packed in suitable containers for shipment, or refined by means of any suitable process.

In the practice of my improved process above described, the following salient features which distinguish the same from processes heretofore employed for a like purpose are to be noted. First, the vegetable matter is not closely confined in a retort or burner, but the chamber is entirely open at its top to the air and the burner employed is of a simple and light construction and can be readily moved from place to place. Secondly, it has heretofore been impossible to recover from sage brush, straw, and like materials, the potassium salts therein contained in commercial quantities. The present invention has for its principal object the recovery of potassium salts from sage brush which grows over vast areas in the western section of the United States, and in such quantities that its recovery will be commercially profitable. Thirdly, and of greatest importance is the addition of sulfur or sulfuric acid to the burning material. By the use of sulfur, it is unnecessary to burn the material in an inclosed chamber to prevent the dissipation of volatile potassium salts

into the atmosphere, as a chemical reaction occurs which converts the potassium from its volatile form into involatile matter. Thus, although the top of the burner is entirely open and oxygen may freely enter thereto, the loss or escape of the potassium salts is effectually prevented.

And lastly, in the practice of the present invention it is not necessary that the material shall be slowly burned under an even or uniform temperature which simply results in a charring of the material, but the material may be burned as rapidly as the nature of the case will permit without a strong forced draft. This is due to the fact that the addition of the sulfur enables me to combine rapidity of combustion with a maximum retention of potassium salts. It will, of course, be manifest that in the practice of the present invention, any desired sulfur containing material may be used, the sulfur being supplied either in a pure or modified state in the form of lump or powdered sulfur, or an acid solution thereof.

From the foregoing, the process and manner of practising the same will be clearly and fully understood. The invention is adapted for the recovery of potassium salts without waste or loss not only from seaweed but sage brush, straw, wood, or any other organic carbonaceous materials as well. As there are no clinkers in the residuary ash, the ashes will readily fall through the grate and they are sifted automatically through the wire screen 14. The burner construction which I have illustrated in the accompanying drawing is, of course, merely tentative, and while well adapted for the purpose in view as it provides a light portable construction, it is manifest that my improved process might be practically performed with various other types of burners. Therefore, in so far as the burner construction is concerned, it is to be understood that I expressly reserve the privilege of varying the construction thereof in any manner which experience or special conditions may indicate to be advisable.

Having thus fully described my invention, what I desire to claim and secure by Letters Patent is:—

1. The process of recovering potassium salts from organic carbonaceous materials which consists in placing the material in an open chamber and incinerating the same, and adding a material which, under the action of heat, will liberate sulfur oxid gases to convert the potassium chlorid in the material into potassium sulfate.

2. The process of recovering potassium salts from organic carbonaceous materials which consists in incinerating the same in an open chamber and under a forced draft, and adding sulfur to liberate sulfur oxid gases which penetrate the material during

the burning and convert the potassium chlorid existing therein into potassium sulfate.

3. The process of recovering potassium salts from organic carbonaceous materials which consists in burning the material in an open-top chamber and under a forced draft and adding sulfur to the burning material to liberate sulfur oxid gases which pen-

trate the material and convert the potassium chlorid in the material into potassium sulfate, and finally sifting the residuary ash.

In testimony whereof I hereunto affix my signature in the presence of two witnesses.

FRANKLIN C. GRIMES.

Witnesses:

LOLA R. ECKHARDT,  
RALPH ECKHARDT.

Copies of this patent may be obtained for five cents each, by addressing the "Commissioner of Patents, Washington, D. C."